

## UNITED STATES PATENT OFFICE

2,524,648

## ELECTRODEPOSITION OF NICKEL

Henry Brown, Detroit, Mich., assignor to The  
Udylite Corporation, Detroit, Mich., a corpora-  
tion of Delaware

No Drawing. Application July 9, 1945,  
Serial No. 604,079

4 Claims. (Cl. 204—49)

1

My invention relates to improvements in the electrodeposition of metals. It is particularly concerned with the utilization of certain addition agents, for the purposes hereinafter stated, in aqueous acidic electroplating baths.

I have discovered that certain substances, hereinafter described in detail, when added to electroplating baths, particularly aqueous acidic electroplating baths such as used for the electrodeposition of nickel, cobalt, iron, zinc, cadmium, copper, antimony, various alloys containing the aforementioned and other metals, and the like, are remarkably effective in the prevention of the formation of pits in the electro-deposited coatings, said pits normally being caused by the adherence of gas bubbles during the electrodeposition of the coating. I have found, further, that this result is accomplished despite the fact that very low concentrations of the addition substances are employed and, still further, that these results are accomplished without causing any significantly appreciable interference with the desired appearance, structure, and character of the plate.

I have also discovered that the addition agents are highly effective independently of whether various organic or inorganic so-called brightening agents are also present in the electrolyte bath. Various addition agents have heretofore been suggested for reducing or eliminating pitting in electrodeposition operations but, at least in most cases, and apart from other deficiencies which they possess, they have proven to be wholly unsatisfactory where the electrodeposition bath contained brighteners. Thus, for example, in baths employed for the electrodeposition of bright nickel, where the brightening agent comprises an aryl sulphonic acid, for example, naphthalene 1,5 disulphonic acid, sodium salt, or sulphonamides or sulphonimides, for example, saccharin, such as are disclosed in my Patent No. 2,191,813, issued February 27, 1940, various suggested anti-pitting agents have proven entirely unsatisfactory. The use of the addition agents in bright plating baths represents but one aspect of my present invention although, to be sure, a highly important one.

The addition agents which I have found to be unusually satisfactory, in accordance with my present invention, can be used in sufficiently low concentrations so as to reduce substantially, or eliminate entirely, pitting of the deposits and, at the same time, they do not interfere to any significantly appreciable extent with the particular cathodic process involved such as reduction of inorganic or organic substances taking place in the process of electrodepositing the coating.

2

This is highly important where the deposited metal is desired not only free from pits but also of maximum ductility and purity and freedom from such inclusions as sulphur, carbon and colloids. It is also of considerable importance in those cases involving bright plating baths, particularly aqueous acid plating baths for the electrodeplating of nickel, which baths contain brighteners such as those mentioned hereinabove, particularly those wherein the brightener is in the form of a soluble compound containing the radical  $-\text{SO}_2\text{N}-$ . As I have pointed out hereinabove, the brightness or brilliance or high luster of the deposits is not adversely affected where the addition agents, to which my present invention relates, are employed.

The novel and highly useful addition agents which accomplish the functions set out hereinabove are, in general, sulpho-monocarboxylic acid esters, particularly, sulpho-fatty acid esters, of water-soluble polyhydric alcohols partially etherified with aliphatic alcohols, particularly fatty alcohols, containing from 8 to 18 carbon atoms. The sulpho-monocarboxylic radical contains from 2 to 6 carbon atoms, the sulphoacetates being particularly satisfactory. My copending application Serial No. 379,950, application February 21, 1941, now Patent 2,389,135, is directed to aliphatic sulpho-mono-carboxylic acid esters of aliphatic alcohols containing from 8 to 18 carbon atoms. My copending application Serial No. 379,951, application February 21, 1941, now Patent 2,389,179, is directed to sulphuric acid esters or sulphates of water-soluble polyhydric alcohols partially esterified with aliphatic carboxylic acids, particularly fatty acids, containing from 8 to 18 carbon atoms. My copending application Serial No. 381,547, application March 3, 1941, now Patent 2,389,180, is directed to sulphocarboxylic acid esters, particularly, sulpho-fatty acid esters, of water-soluble polyhydric alcohols partially esterified with aliphatic carboxylic acids, particularly fatty acids, containing from 8 to 18 carbon atoms.

Various of the addition agents utilized in accordance with the present invention may be represented by the formula



where R is an alkyl radical containing from 8 to 18 carbon atoms, M is a cation such as hydrogen, alkali metals or a metal corresponding to that of the metal being electrodeposited, for example, nickel, X is the residue of an aliphatic polyhydric alcohol, Y is the carbon-hydrogen

residue of a sulpho-monocarboxylic acid, and  $v$  and  $w$  are small whole numbers such as 1 or 2.

The polyethylene glycol alkyl ether sulpho-monocarboxylic acid ester addition agents, whose use represents a particularly preferred embodiment of my present invention, may be represented by the formula



where R, M and Y are the same as in the immediately preceding formula, and  $n$  is a whole number such as 1, 2, 3, 4 or more, preferably 2 to 4.

Illustrative examples of addition agents which may be utilized in accordance with my invention and in the concentrations which are, in general, preferred, are shown in Table I:

Table I

| Anion                                                                                                                        | Cation                                     | Conc.,<br>grams/liter |
|------------------------------------------------------------------------------------------------------------------------------|--------------------------------------------|-----------------------|
| (1) $CH_3-(CH_2)_9-O-CH_2-CH_2-O-OC-CH_2-SO_3^-$<br>(Decyl ether of ethylene glycol sulphoacetate)                           | $H^+$ , $Na^+$ or metal of bath being used | 0.1-0.5               |
| (2) $CH_3-(CH_2)_{11}-O-CH_2-CH_2-O-OC-CH_2-SO_3^-$<br>(Lauryl ether of ethylene glycol sulphoacetate)                       | do                                         | 0.1-0.5               |
| (3) $CH_3-(CH_2)_{11}-O-CH_2-OH-CH_2-O-OC-CH_2-SO_3^-$<br>$OH$<br>(Lauryl mono-ether of glycerol mono-sulphoacetate)         | do                                         | 0.1-0.5               |
| (4) $CH_3-(CH_2)_7-O-C_2H_4-O-C_2H_4-O-OC-CH_2-SO_3^-$<br>(Octyl ether of diethylene glycol sulphoacetate)                   | do                                         | 0.1-0.5               |
| (5) $CH_3-(CH_2)_{13}-O-C_2H_4-(O-C_2H_4)_2-O-OC-CH_2-SO_3^-$<br>(Myristyl ether of tetraethylene glycol sulphoacetate)      | do                                         | 0.1-0.5               |
| (6) $CH_3-(CH_2)_9-O-CH_2-CH_2-O-OC-CH_2-CH_2-SO_3^-$<br>(Decyl ether of ethylene glycol sulphopropionate)                   | do                                         | 0.1-0.5               |
| (7) $CH_3-(CH_2)_{11}-(O-CH_2-CH_2-CH_2)_2-O-OC-CH_2-SO_3^-$<br>$OH$<br>(Lauryl mono-ether of diglycerol mono-sulphoacetate) | do                                         | 0.1-0.5               |

The water-soluble aliphatic polyhydric alcohols, the specific ethers of which, in the form of sulpho-monocarboxylic acid esters, comprise the addition agents of my present invention, may be selected from a large class and include, for example, glycerin; glycols such as ethylene glycol, propylene glycol, trimethylene glycol, butylene glycol, and the like; polyglycols such as diethylene glycol, triethylene glycol, tetraethylene glycol, and the like; pentaerythritol; dipentaerythritol; polyglycerols such as diglycerol, triglycerol, tetraglycerol and mixtures thereof; carbohydrates and sugars such as dextrose, sucrose, and maltose; and sugar alcohols such as arabitol, mannitol, sorbitol, dulcitol, mannanol and sorbitan, and the like.

The aliphatic alcohols with which the aforementioned or similar water-soluble aliphatic polyhydric alcohols are etherified may also be selected from a large group including, by way of illustration, straight chain and branched chain alcohols such as octyl alcohol, nonyl alcohol, decyl alcohol, undecyl alcohol, lauryl alcohol, myristyl alcohol, cetyl alcohol, oleyl alcohol, linoleyl alcohol, stearyl alcohol, ricinoleyl alcohol, and palmitoleyl alcohol, and the like; branched chain octyl, decyl, dodecyl, tetradecyl, hexadecyl and octadecyl aliphatic alcohols as, for example, 2-ethyl hexanol-1; 2-n butyl octanol-1; 2-butyl tetra-decanol-1; 7-ethyl 2-methylundecanol-4; 3,9 diethyltridecanol-6; 3-methylheptanol-2; 5,11 diethylpentadecanol-8; 5-ethylnonanol-2; 7-ethyl-2-methyltridecanol-4; 9-ethyl-5-methyl-

tridecanol-6; 5-ethyltridecanol-8; 3-ethylheptanol-6; 3-ethyl-8-methylnonanol-6; 3-ethylundecanol-6; and 2-methylnonanol-4. I prefer particularly to use the straight chain, unsubstituted fatty alcohols containing from 8 to 12 carbon atoms. Any of the aliphatic alcohols listed hereinabove may be etherified with any of the listed polyhydric alcohols to form partial ethers, especially mono-ethers, the sulpho-monocarboxylic acid esters, particularly the mono-esters, of which comprise the addition agents used in accordance with the present invention.

The sulpho-monocarboxylic acid radical, as pointed out hereinabove, should contain not more than six carbon atoms. Especially satisfactory are the sulphoacetates, although sulphopropion-

ates, sulphobutyrate, sulphovalerates, sulphoacrylates, and the like may also be utilized.

It will be understood that the sulpho-monocarboxylic acid radical is linked to the remainder of the molecule of the addition agent through an hydroxy group of the aliphatic polyhydric alcohol radical. As indicated above, the molecule of the addition agent may contain one or more aliphatic or fatty alcohol radicals and one or more sulpho-monocarboxylic acid groups. Of especial utility are the sulphoacetates of glycerin and glycol partial ethers of decyl and lauryl alcohols or coconut oil mixed fatty alcohols or special fractions particularly high in content of decyl or lauryl alcohols.

The addition agents are utilized preferably in the form of their free acids or their alkali metal salts or in the form of a salt of the metal to be electrodeposited. In most cases, it is preferable to utilize the sodium salt.

The addition agents are employed in concentrations of the general order of about 0.05 to about 0.5 gram per liter of electrolyte solution, from about 0.1 to about 0.3 gram per liter of electrolyte solution being most satisfactory in the usual case. More addition agent may be utilized but it is, in general, uneconomic to do so and fully satisfactory results are obtained in practically all cases with the preferred range set out hereinabove.

It will be understood that the addition agents utilized should be soluble in the electrolyte solution at least to such an extent as to fall within the general range as set out hereinabove. In

general, the solubility of the addition agents in the electrolyte solutions decreases with the increase of carbon atoms in the alkyl chain of the addition agents and, therefore, lower concentrations of such addition agents may be used. Conversely, higher concentrations, generally speaking, of those addition agents should be used where the number of carbon atoms in the alkyl chain is around 8 or 10 carbon atoms.

Table II sets forth various examples of plating baths with which the addition agents of the present invention may be used effectively to prevent or inhibit pitting. It will be understood that these examples are merely illustrative and are not to be taken as limitative of my invention, it being understood that, in general, the novel teachings of my invention may be utilized in connection with plating baths wherein the addition agents are soluble in the electrolyte solutions to the extent necessary to accomplish the desired results, and wherein said addition agents are not hydrolyzed or otherwise decomposed or modified to an extent sufficient to interfere with their functioning. In general, the addition agents are particularly effective in aqueous acidic electroplating baths wherein the pH of the bath is of the order of about 2 to about 6.

Table II

[In each bath 0.1-0.5 gram/liter or 0.01-0.07 oz./gal. of monolauryl ether of diethylene glycol sulfoacetate, sodium salt.]

| Nickel (white)                                                                        | conc., oz./gal. | Nickel (white)                                                 | conc., oz./gal. |
|---------------------------------------------------------------------------------------|-----------------|----------------------------------------------------------------|-----------------|
| NiSO <sub>4</sub> .6-7H <sub>2</sub> O                                                | 30-40           | NiCl <sub>2</sub> .6H <sub>2</sub> O                           | 30-40           |
| NiCl <sub>2</sub> .6H <sub>2</sub> O                                                  | 8               | H <sub>3</sub> BO <sub>3</sub>                                 | 5               |
| H <sub>3</sub> BO <sub>3</sub>                                                        | 5               | Temp. 70-150° F                                                |                 |
| Temp. 100-150° F                                                                      |                 | pH=4.0-5.5                                                     |                 |
| pH=4.0-5.5                                                                            |                 | Cathode C. D., 5-150 amp./ft. <sup>2</sup>                     |                 |
| Cathode C. D., 5-75 amp./ft. <sup>2</sup>                                             |                 |                                                                |                 |
| Nickel (Bright)                                                                       | conc., oz./gal. | Cobalt                                                         | conc., oz./gal. |
| NiSO <sub>4</sub> .6-7H <sub>2</sub> O                                                | 30-40           | CoSO <sub>4</sub> .7H <sub>2</sub> O                           | 30-40           |
| NiCl <sub>2</sub> .6H <sub>2</sub> O                                                  | 8               | CoCl <sub>2</sub> .6H <sub>2</sub> O                           | 8               |
| H <sub>3</sub> BO <sub>3</sub>                                                        | 5               | H <sub>3</sub> BO <sub>3</sub>                                 | 5               |
| C <sub>6</sub> H <sub>5</sub> -SO <sub>2</sub> NH <sub>2</sub>                        | 0.3             | (NH <sub>4</sub> ) <sub>2</sub> SO <sub>4</sub>                | 0.2             |
| ZnSO <sub>4</sub> .7H <sub>2</sub> O                                                  | 0.1             | Temp. 70-120° F                                                |                 |
| Temp. 100-150° F                                                                      |                 | pH=3.5-5.5                                                     |                 |
| pH=3.5-5.5                                                                            |                 | Cathode C. D., 20-200 amp./ft. <sup>2</sup>                    |                 |
| Cathode C. D., 15-75 amp./ft. <sup>2</sup>                                            |                 |                                                                |                 |
| Nickel-Cobalt (Bright)                                                                | conc., oz./gal. | Zinc                                                           | conc., oz./gal. |
| NiSO <sub>4</sub> .6-7H <sub>2</sub> O                                                | 32              | ZnSO <sub>4</sub> .7H <sub>2</sub> O                           | 30-40           |
| CoSO <sub>4</sub> .7H <sub>2</sub> O                                                  | 8               | Zn(C <sub>2</sub> H <sub>5</sub> O <sub>2</sub> ) <sub>2</sub> | 4               |
| NiCl <sub>2</sub> .6H <sub>2</sub> O                                                  | 6               | Al <sub>2</sub> (SO <sub>4</sub> ) <sub>3</sub>                | 2               |
| H <sub>3</sub> BO <sub>3</sub>                                                        | 5               | Temp. 100-150° F                                               |                 |
| HCHO                                                                                  | 0.15            | pH=4.0-5.5                                                     |                 |
| Temp. 100-150° F                                                                      |                 | Cathode C. D., 10-50 amp./ft. <sup>2</sup>                     |                 |
| pH=4.0-5.5                                                                            |                 |                                                                |                 |
| Cathode C. D., 5-100 amp./ft. <sup>2</sup>                                            |                 |                                                                |                 |
| Iron                                                                                  | conc., oz./gal. | Copper                                                         | conc., oz./gal. |
| FeCl <sub>2</sub>                                                                     | 40              | CuSO <sub>4</sub> .5H <sub>2</sub> O                           | 30-40           |
| CaCl <sub>2</sub> .6H <sub>2</sub> O                                                  | 20              | Cu(C <sub>2</sub> H <sub>5</sub> O <sub>2</sub> ) <sub>2</sub> | 4               |
| Temp. 100-150° F                                                                      |                 | Temp. 70-150° F                                                |                 |
| pH=3.5-5.0                                                                            |                 | pH=3.0-5.0                                                     |                 |
| Cathode C. D., 10-100 amp./ft. <sup>2</sup>                                           |                 | Cathode C. D., 10-50 amp./ft. <sup>2</sup>                     |                 |
| Iron                                                                                  | conc., oz./gal. |                                                                |                 |
| FeSO <sub>4</sub> .(NH <sub>4</sub> ) <sub>2</sub> SO <sub>4</sub> .6H <sub>2</sub> O | 24-32           |                                                                |                 |
| Temp.—Room to 160° F                                                                  |                 |                                                                |                 |
| pH=4-5                                                                                |                 |                                                                |                 |
| Cathode C. D., 5-100 amp./ft. <sup>2</sup>                                            |                 |                                                                |                 |

While, in the examples listed hereinabove in Table II, I have disclosed the use of the sodium salt of the mono-lauryl ether of diethylene glycol sulfoacetate as the addition agent, it will be understood that others of the addition agents which I have disclosed may be substituted therefor without in any manner departing from the spirit and teachings of my invention.

It will be understood that, from time to time, 10 more addition agent should be added to replenish that which is lost by "drag-out" or which may possibly be changed, in some manner or other, during the electrodeposition process.

This application is a continuation-in-part of 15 my prior application, Serial No. 381,547, filed March, 3, 1941.

What I claim as new and desire to protect by Letters Patent of the United States is:

1. In a process of electrodepositing nickel, the 20 step which comprises electrolyzing an aqueous acid nickel solution of a material selected from the group consisting of nickel sulphate, nickel chloride, and mixtures thereof, said aqueous solution also having dissolved therein a minor proportion of at least .05 gram per liter of a soluble aliphatic sulpho-monocarboxylic acid ester of a water-soluble aliphatic polyhydric alcohol the 25

2. In a process of electrodepositing nickel, the

3. In a process of electrodepositing nickel, the

4. In a process of electrodepositing nickel, the

5. In a process of electrodepositing nickel, the

6. In a process of electrodepositing nickel, the

7. In a process of electrodepositing nickel, the

8. In a process of electrodepositing nickel, the

9. In a process of electrodepositing nickel, the

10. In a process of electrodepositing nickel, the

11. In a process of electrodepositing nickel, the

12. In a process of electrodepositing nickel, the

13. In a process of electrodepositing nickel, the

14. In a process of electrodepositing nickel, the

15. In a process of electrodepositing nickel, the

16. In a process of electrodepositing nickel, the

17. In a process of electrodepositing nickel, the

18. In a process of electrodepositing nickel, the

19. In a process of electrodepositing nickel, the

20. In a process of electrodepositing nickel, the

21. In a process of electrodepositing nickel, the

22. In a process of electrodepositing nickel, the

23. In a process of electrodepositing nickel, the

24. In a process of electrodepositing nickel, the

25. In a process of electrodepositing nickel, the

26. In a process of electrodepositing nickel, the

27. In a process of electrodepositing nickel, the

28. In a process of electrodepositing nickel, the

29. In a process of electrodepositing nickel, the

30. In a process of electrodepositing nickel, the

31. In a process of electrodepositing nickel, the

32. In a process of electrodepositing nickel, the

33. In a process of electrodepositing nickel, the

34. In a process of electrodepositing nickel, the

35. In a process of electrodepositing nickel, the

36. In a process of electrodepositing nickel, the

37. In a process of electrodepositing nickel, the

38. In a process of electrodepositing nickel, the

39. In a process of electrodepositing nickel, the

40. In a process of electrodepositing nickel, the

41. In a process of electrodepositing nickel, the

42. In a process of electrodepositing nickel, the

43. In a process of electrodepositing nickel, the

44. In a process of electrodepositing nickel, the

45. In a process of electrodepositing nickel, the

46. In a process of electrodepositing nickel, the

47. In a process of electrodepositing nickel, the

48. In a process of electrodepositing nickel, the

49. In a process of electrodepositing nickel, the

50. In a process of electrodepositing nickel, the

51. In a process of electrodepositing nickel, the

52. In a process of electrodepositing nickel, the

53. In a process of electrodepositing nickel, the

54. In a process of electrodepositing nickel, the

55. In a process of electrodepositing nickel, the

56. In a process of electrodepositing nickel, the

57. In a process of electrodepositing nickel, the

58. In a process of electrodepositing nickel, the

59. In a process of electrodepositing nickel, the

60. In a process of electrodepositing nickel, the

61. In a process of electrodepositing nickel, the

62. In a process of electrodepositing nickel, the

63. In a process of electrodepositing nickel, the

64. In a process of electrodepositing nickel, the

65. In a process of electrodepositing nickel, the

66. In a process of electrodepositing nickel, the

67. In a process of electrodepositing nickel, the

68. In a process of electrodepositing nickel, the

69. In a process of electrodepositing nickel, the

70. In a process of electrodepositing nickel, the

71. In a process of electrodepositing nickel, the

72. In a process of electrodepositing nickel, the

73. In a process of electrodepositing nickel, the

74. In a process of electrodepositing nickel, the

75. In a process of electrodepositing nickel, the

76. In a process of electrodepositing nickel, the

77. In a process of electrodepositing nickel, the

78. In a process of electrodepositing nickel, the

79. In a process of electrodepositing nickel, the

80. In a process of electrodepositing nickel, the

81. In a process of electrodepositing nickel, the

82. In a process of electrodepositing nickel, the

83. In a process of electrodepositing nickel, the

84. In a process of electrodepositing nickel, the

85. In a process of electrodepositing nickel, the

86. In a process of electrodepositing nickel, the

87. In a process of electrodepositing nickel, the

88. In a process of electrodepositing nickel, the

89. In a process of electrodepositing nickel, the

90. In a process of electrodepositing nickel, the

91. In a process of electrodepositing nickel, the

92. In a process of electrodepositing nickel, the

93. In a process of electrodepositing nickel, the

94. In a process of electrodepositing nickel, the

95. In a process of electrodepositing nickel, the

96. In a process of electrodepositing nickel, the

97. In a process of electrodepositing nickel, the

98. In a process of electrodepositing nickel, the

99. In a process of electrodepositing nickel, the

100. In a process of electrodepositing nickel, the

101. In a process of electrodepositing nickel, the

102. In a process of electrodepositing nickel, the

103. In a process of electrodepositing nickel, the

104. In a process of electrodepositing nickel, the

105. In a process of electrodepositing nickel, the

106. In a process of electrodepositing nickel, the

107. In a process of electrodepositing nickel, the

108. In a process of electrodepositing nickel, the

109. In a process of electrodepositing nickel, the

110. In a process of electrodepositing nickel, the

111. In a process of electrodepositing nickel, the

112. In a process of electrodepositing nickel, the

113. In a process of electrodepositing nickel, the

114. In a process of electrodepositing nickel, the

115. In a process of electrodepositing nickel, the

116. In a process of electrodepositing nickel, the

117. In a process of electrodepositing nickel, the

118. In a process of electrodepositing nickel, the

119. In a process of electrodepositing nickel, the

120. In a process of electrodepositing nickel, the

121. In a process of electrodepositing nickel, the

122. In a process of electrodepositing nickel, the

123. In a process of electrodepositing nickel, the

124. In a process of electrodepositing nickel, the

125. In a process of electrodepositing nickel, the

126. In a process of electrodepositing nickel, the

127. In a process of electrodepositing nickel, the

128. In a process of electrodepositing nickel, the

129. In a process of electrodepositing nickel, the

130. In a process of electrodepositing nickel, the

131. In a process of electrodepositing nickel, the

132. In a process of electrodepositing nickel, the

133. In a process of electrodepositing nickel, the

134. In a process of electrodepositing nickel, the

135. In a process of electrodepositing nickel, the

136. In a process of electrodepositing nickel, the

137. In a process of electrodepositing nickel, the

138. In a process of electrodepositing nickel, the

139. In a process of electrodepositing nickel, the

140. In a process of electrodepositing nickel, the

141. In a process of electrodepositing nickel, the

142. In a process of electrodepositing nickel, the

143. In a process of electrodepositing nickel, the

144. In a process of electrodepositing nickel, the

145. In a process of electrodepositing nickel, the

146. In a process of electrodepositing nickel, the

147. In a process of electrodepositing nickel, the

148. In a process of electrodepositing nickel, the

149. In a process of electrodepositing nickel, the

150. In a process of electrodepositing nickel, the

151. In a process of electrodepositing nickel, the

152. In a process of electrodepositing nickel, the

153. In a process of electrodepositing nickel, the

154. In a process of electrodepositing nickel, the

155. In a process of electrodepositing nickel, the

156. In a process of electrodepositing nickel, the

157. In a process of electrodepositing nickel, the

158. In a process of electrodepositing nickel, the

159. In a process of electrodepositing nickel, the

160. In a process of electrodepositing nickel, the

161. In a process of electrodepositing nickel, the

162. In a process of electrodepositing nickel, the

163. In a process of electrodepositing nickel, the

164. In a process of electrodepositing nickel, the

165. In a process of electrodepositing nickel, the

166. In a process of electrodepositing nickel, the

167. In a process of electrodepositing nickel, the

168. In a process of electrodepositing nickel, the

169. In a process of electrodepositing nickel, the

170. In a process of electrodepositing nickel, the

171. In a process of electrodepositing nickel, the

172. In a process of electrodepositing nickel, the

173. In a process of electrodepositing nickel, the

174. In a process of electrodepositing nickel, the

175. In a process of electrodepositing nickel, the

the group consisting of nickel sulphate, nickel chloride, and mixtures thereof, said aqueous solution also having dissolved therein a minor proportion of at least .05 gram per liter of the lauryl mono-ether of diethylene glycol sulphoacetate.

3. A bath for the electrodeposition of nickel consisting essentially of an aqueous acid solution of a material selected from the group consisting of nickel sulphate, nickel chloride, and mixtures thereof, and a minor proportion of at least .05 gram per liter of a soluble aliphatic sulpho-fatty acid ester of a water-soluble aliphatic polyhydric alcohol the hydrogen of at least one hydroxy group of which is replaced by an alkyl radical containing from 8 to 18 carbon atoms, the sulpho-fatty acid radical containing from 2 to 6 carbon atoms inclusive. 15

4. A bath for the electrodeposition of nickel

consisting essentially of an aqueous acid solution of a material selected from the group consisting of nickel sulphate, nickel chloride, and mixtures thereof, and a minor proportion of at least .05 gram per liter of a mono-sulphoacetate of a lauryl mono-ether of a glycol.

HENRY BROWN.

#### REFERENCES CITED

10 The following references are of record in the file of this patent:

#### UNITED STATES PATENTS

| Number    | Name  | Date          |
|-----------|-------|---------------|
| 2,389,135 | Brown | Nov. 20, 1945 |
| 2,389,179 | Brown | Nov. 20, 1945 |
| 2,389,180 | Brown | Nov. 20, 1945 |
| 2,389,181 | Brown | Nov. 20, 1945 |